

## UNITED STATES PATENT OFFICE

2,378,992

## ARTICLES FOR USE AT LOW TEMPERATURES

Russell Franks, Niagara Falls, N. Y., assignor to  
Electro Metallurgical Company, a corporation  
of West Virginia

No Drawing. Application January 16, 1943,  
Serial No. 472,597

9 Claims. (CL. 75—123)

This invention relates to steel articles for use at low temperatures.

A demand exists in industry for steels for use in the fabrication of apparatus for use at low temperatures, for example for refrigerating equipment or for apparatus used in the handling of liquefied gases such as oxygen, nitrogen, or air. Many steels which have excellent strength and toughness at normal atmospheric temperatures become brittle when exposed to temperatures below zero on the centigrade scale, and few ferrous materials have the requisite toughness to withstand shock at the exceedingly low temperatures encountered in handling liquefied air or oxygen. Stainless steels of the type containing about 18% chromium and 8% nickel have excellent toughness even at temperatures in the neighborhood of  $-183^{\circ}$  C., and have been widely used in liquid oxygen equipment, but these steels are relatively expensive. Although nonferrous metals and alloys are not as susceptible as ferrous materials to loss of toughness at low temperatures, in general, their strength is not great.

It is the chief object of this invention to provide articles for use at low temperatures which articles are composed of steel which possesses the ability to withstand shock at very low temperatures.

The invention by means of which this object is achieved is based on the discovery that austenitic manganese steels which contain substantial proportions of manganese within certain narrow, critical limits and a minor proportion of at least one austenite-stabilizing element selected from the group consisting of nickel and copper, with or without chromium in a proportion up to 16%, have the ability to withstand shock at sub-zero temperatures. The invention comprises articles for use at low temperatures composed of such steels.

More specifically, the invention comprises articles for use at low temperatures, which articles are composed of steel containing about 15% to 20% manganese, 0.2% to 8% of at least one austenite-stabilizing element selected from the group consisting of nickel and copper, up to about 16% chromium and the remainder chiefly iron. Preferably, the steel contains both nickel and copper. If nickel alone is used, the steel should contain about 0.5% to 5% (preferably 1% to 5%) of this element. If copper alone is used, the steel should contain about 0.25% to 2% of this element, but if both copper and nickel are used, the copper content may be as high as 3%. Ordinarily, the presence of more than 3% of copper should be avoided because of the detrimental effect of copper on the hot working properties of the steel.

The presence of chromium in the steel not only

improves its toughness at low temperatures but also enhances its resistance to corrosion. Where corrosion-resistance is not important, chromium may be omitted altogether, but in such case the sum of the nickel and copper content should be at least 4%, and preferably at least 5%, of the steel to secure the desired low temperature toughness. Where resistance merely to progressive rusting is desired, the steel should contain about 0.25% to 8%, preferably 1% to 4%, chromium. In steels containing chromium in this range, the sum of the nickel and copper contents need not be as high as when chromium is not present in the steel. Where a high degree of resistance to corrosion is required of the articles of the invention in addition to low temperature toughness, the steel of which they are composed should contain about 8% to 16% chromium, and in such case for the greatest degree of toughness at low temperature, the steel should contain about 0.2% to 3% nickel or about 0.2% to 2.25% copper or both nickel and copper. A preferred lower limit for nickel or copper or both is about 0.25%. Generally, best results are obtained in all of these steels if nickel or both nickel and copper are present, but in the higher chromium steels a small proportion of either will suffice.

The carbon content of the steel of which the articles of the invention are composed should not exceed about 0.5% and is preferably about 0.01% to 0.35%. Nitrogen in a proportion up to about 0.15% and phosphorus up to about 0.4% (preferably not more than about 0.2%) may be present in the steel, nitrogen in particular having a beneficial effect on its toughness. There will also ordinarily be normal percentages of residual deoxidizers, scavengers and grain refiners such as silicon and calcium present in the steel.

The articles of the invention should be annealed before exposure to low temperatures, suitably by heating them at a temperature above about  $900^{\circ}$  C. and then rapidly cooling them in water or air.

The toughness at low temperature of austenitic manganese steels containing various amounts of nickel, copper, and chromium is illustrated by the test data set forth in Table I. In this table the impact resistance at room temperature and at  $-183^{\circ}$  C. of the steels as determined in the standard Izod impact test is given in foot pounds. The specimens tested at  $-183^{\circ}$  C. were cooled to that temperature by immersing them in liquid air for one-half to one hour and then were quickly transferred to the impact machine and tested. Before testing, all specimens were annealed by heating them for ten to twenty minutes at  $1000^{\circ}$  C. to  $1050^{\circ}$  C. and then cooling them in air.

Table I

| Composition (remainder iron) |            |            |            |           | Impact resistance |          |
|------------------------------|------------|------------|------------|-----------|-------------------|----------|
| Percent Mn                   | Percent Ni | Percent Cu | Percent Cr | Percent C | Room temp.        | -183° C. |
| 14                           | Nil        | Nil        | Nil        | 0.30      | 8                 | 0.75     |
| 16.5                         | Nil        | Nil        | Nil        | 0.20      | 32                | 3        |
| 18                           | Nil        | Nil        | Nil        | 0.30      | 65                | 2        |
| 17                           | 2.0        | Nil        | Nil        | 0.29      | 96                | 16       |
| 16                           | 4.5        | Nil        | Nil        | 0.30      | 94                | 30       |
| 17                           | 2          | 1          | Nil        | 0.20      | 103               | 20       |
| 16.5                         | 2          | 2          | Nil        | 0.10      | 90                | 46       |
| 16                           | 2          | 2          | Nil        | 0.40      | 70                | 32       |
| 17                           | 3          | 1          | Nil        | 0.10      | 107               | 41       |
| 16                           | 2          | 1          | 3          | 0.20      | 102               | 28       |
| 17                           | 2          | 2          | 3          | 0.10      | 97                | 63       |
| 17.5                         | 2          | Nil        | 5.07       | 0.20      | 93                | 42       |
| 16.5                         | 0.54       | Nil        | 12.9       | 0.15      | 105               | 60       |
| 16.5                         | 1.10       | Nil        | 13.2       | 0.15      | 100               | 67       |
| 16.2                         | 2.10       | Nil        | 13.2       | 0.14      | 100               | 90       |
| 16.5                         | Nil        | 0.75       | 12.8       | 0.13      | 100               | 67       |
| 16.5                         | 0.58       | 0.64       | 12.9       | 0.13      | 100               | 64       |
| 16.3                         | 1.10       | 0.60       | 13.0       | 0.12      | 98                | 78       |

The data in Table I show the drop in toughness of the plain high manganese steel at low temperature and that the addition of copper or nickel or both markedly improves the toughness of high manganese steel at low temperature. Even further improvement is shown by steels containing chromium in addition to nickel or copper or both.

Tensile test data set forth in Table II below demonstrate that the ductility of high manganese steel, as measured by the percentage elongation in a two inch gauge length, is enhanced by the presence of one or both of the elements nickel and copper, with or without chromium.

Table II

| Composition (remainder iron) |            |            |            |           | Yield strength, p. s. i. | Tensile strength, p. s. i. | Percent el. in 2" |
|------------------------------|------------|------------|------------|-----------|--------------------------|----------------------------|-------------------|
| Percent Mn                   | Percent Ni | Percent Cu | Percent Cr | Percent C |                          |                            |                   |
| 14                           | Nil        | Nil        | Nil        | 0.30      | 38,500                   | 110,300                    | 14                |
| 16.5                         | Nil        | Nil        | Nil        | 0.20      | 36,100                   | 127,300                    | 24                |
| 17                           | 2          | Nil        | Nil        | 0.29      | 35,000                   | 127,000                    | 60                |
| 17                           | 4.5        | Nil        | Nil        | 0.28      | 31,800                   | 112,900                    | 62                |
| 16.5                         | 2          | 1          | Nil        | 0.15      | 29,500                   | 111,300                    | 59                |
| 16.5                         | 2          | 2          | Nil        | 0.10      | 28,000                   | 106,700                    | 62                |
| 16                           | 2          | 2          | Nil        | 0.40      | 37,100                   | 138,000                    | 69                |
| 16                           | 2          | 1          | 3          | 0.20      | 35,100                   | 120,400                    | 61                |
| 16                           | 2          | 2          | 3          | 0.13      | 27,600                   | 136,500                    | 65                |
| 17.5                         | 2          | Nil        | 5.07       | 0.20      | 40,700                   | 120,000                    | 53                |
| 16.5                         | Nil        | 0.75       | 12.8       | 0.13      | 36,000                   | 123,000                    | 63                |
| 16.5                         | 0.54       | Nil        | 12.9       | 0.12      | 36,000                   | 128,500                    | 62                |
| 16.5                         | 1.1        | Nil        | 13.2       | 0.15      | 38,500                   | 124,500                    | 67                |
| 16.3                         | 1.1        | 0.6        | 13         | 0.12      | 35,000                   | 108,000                    | 63                |
| 16.2                         | 2.1        | Nil        | 13.2       | 0.14      | 36,000                   | 110,000                    | 63                |
| 16.5                         | 2          | 1.5        | 12         | 0.10      | 31,000                   | 101,500                    | 58                |

The test data shown in Table II were obtained on standard tensile test specimens at room temperature, the yield strength at 0.2% offset being determined in accordance with United States Navy Department specification No. 47S21. In the table "yield strength p. s. i." represents the yield strength in tension measured at 0.2% permanent set in pounds per square inch; "tensile strength p. s. i." represents ultimate tensile strength in pound per square inch; and "percent el." represents percentage elongation of the tensile test specimen to rupture in an initial gauge length of two inches.

The high manganese steel containing nickel or copper or chromium or any of these elements may be readily welded by known fusion welding processes. Welds made in the steel with rods of the same analysis as the plate have good toughness and strength. Even tougher welds may be obtained by welding the steel with austenitic stain-

less steel welding rods containing about 5% to 30% chromium and 5% to 30% nickel, for instance, using rods containing 18% chromium and 8% nickel or 24% chromium and 12% nickel or 25% chromium and 20% nickel.

I claim:

1. A steel article for use at low temperatures, which article is composed of a steel containing about 15% to 20% manganese to render said

10 steel austenitic, about 0.2% to 8% of at least one austenite-stabilizing element selected from the group consisting of nickel and copper, the copper content not exceeding about 3% of the steel, 0.01% to 0.5% carbon and the remainder iron and

15 incidental elements having to substantial adverse effect on the low temperature toughness of said steel.

2. A steel article for use at low temperatures, which article is composed of a steel containing about 15% to 20% manganese to render said

20 steel austenitic, about 0.2% to 8% of at least one austenite-stabilizing element selected from the group consisting of nickel and copper, the copper content not exceeding about 3% of the steel, up to about 16% chromium, 0.01% to 0.5% carbon and the remainder substantially all iron.

3. A steel article for use at low temperatures, which article is composed of a steel containing about 15% to 20% manganese, about 0.5% to 5%

30 nickel, 0.01% to 0.5% carbon and the remainder substantially all iron.

4. A steel article for use at low temperatures, which article is composed of a steel containing about 15% to 20% manganese, about 0.2% to 8% of at least one austenite-stabilizing element selected from the group consisting of nickel and copper, the copper content not exceeding 3% of the steel, about 0.25% to 8% chromium, 0.01% to 0.5% carbon and the remainder substantially all iron.

5. A steel article for use at low temperatures, which article is composed of a steel containing about 15% to 20% manganese, 1% to 5% nickel, 0.25% to 2% copper, 0.25% to 8% chromium, 45 0.01% to 0.5% carbon and the remainder substantially all iron.

6. A steel article for use at low temperatures, which article is composed of a steel containing about 15% to 20% manganese, 1% to 5% nickel, 50 0.25% to 2% copper, 1% to 4% chromium, 0.01% to 0.35% carbon and the remainder substantially all iron.

7. A steel article for use at low temperatures, which article is composed of a steel containing about 15% to 20% manganese, 0.2% to 3% nickel, 55 0.2% to 2.25% copper, 8% to 16% chromium, 0.01% to 0.5% carbon and the remainder substantially all iron.

8. A steel article resistant to progressive rusting which in its normal use is required to withstand shock at temperatures below zero on the centigrade scale, which article is composed of a steel containing about 15% to 20% manganese, 0.25% to 5% nickel, 0.25% to 2% copper, 0.25% to 8% chromium, 60 0.01% to 0.5% carbon, the remainder substantially all iron.

9. A corrosion-resistant steel article which in its normal use is required to withstand shock at temperatures below zero on the centigrade scale, which article is composed of a steel containing about 15% to 20% manganese, 0.25% to 3% nickel, 0.25% to 2.25% copper, 8% to 16% chromium, 65 0.01% to 0.5% carbon, the remainder substantially all iron.

CERTIFICATE OF CORRECTION.

Patent No. 2,378,992.

June 26, 1945.

RUSSELL FRANKS.

It is hereby certified that error appears in the printed specification of the above numbered patent requiring correction as follows: Page 2, first column, line 31, for "ducitility" read --ductility--; line 65, for "pound" read --pounds--; and second column, line 15, for "having to" read --having no--; and that the said Letters Patent should be read with this correction therein that the same may conform to the record of the case in the Patent Office.

Signed and sealed this 2nd day of October, A. D. 1945.

Leslie Frazer

(Seal)

First Assistant Commissioner of Patents.